

April 24, 1962

D. A. NEWMAN

3,031,327

METHOD OF PREPARING TRANSFER SHEETS

Filed Nov. 20, 1959

Fig. 1



Fig. 2



INVENTOR.

Douglas A. Newman  
BY

Johnson and Kline  
ATTORNEYS

## 1

3,031,327

**METHOD OF PREPARING TRANSFER SHEETS**  
Douglas A. Newman, Glen Cove, N.Y., assignor to Columbia Ribbon and Carbon Manufacturing Co., Inc., Glen Cove, N.Y., a corporation of New York  
Filed Nov. 20, 1959, Ser. No. 854,342  
11 Claims. (Cl. 117—36.4)

This invention relates to a new method of preparing novel transfer sheets and ribbons.

Conventional carbon papers have been known for many years and are the most common transfer sheets in use today. These sheets are prepared by coating paper with a layer of melted wax-carrying pigment. Upon cooling, there results a transfer sheet carrying a layer of pressure-transferable wax having homogeneously dispersed therein the pigment, such as carbon black or graphite.

It is recognized that these known carbon papers have many serious disadvantages. Because of the homogeneous distribution of the pigment throughout the wax layer, the transfer sheet is dirty-to-the-touch and thus must be handled by the user with extreme care. It is also a problem in that the transferred image such as typing or writing is likewise dirty-to-the-touch and becomes smudged upon ordinary handling.

Still another important disadvantage of these known carbon sheets is the large amount of pigment which must be used, most of which is wasted.

It is an object of the present invention to prepare transfer sheets and ribbons of the carbon paper type which have a light colored appearance and which are clean-to-the-touch. The foundation may be paper or any plastic film such as cellulose acetate, cellophane, polyethylene terephthalate (Mylar), vinyl polymers, etc.

It is another object of the present invention to prepare carbon papers and ribbons which transfer smudge-proof images of colored or magnetic pigments.

It is a further object of the present invention to prepare carbon papers and ribbons using less pigment than heretofore possible.

These and other objects are accomplished according to the present invention.

In the drawing:

FIGURE 1 is a diagrammatic cross-section view, to an enlarged scale, of the transfer sheets of the present invention.

FIG. 2 is a diagrammatic cross-section view, to an enlarged scale, of a copy sheet carrying an image transferred from the present transfer sheets.

I have found that the many difficulties existing through the use of conventional carbon paper may be avoided and that cleaner and better-appearing transfer sheets and ribbons may be prepared according to the present discovery.

This invention is accomplished by applying a pigment solution or dispersion to the surface of any conventional frangible wax layer carried upon a foundation sheet 10 and heating the mass to the softening or fusion temperature of the wax whereby the liquid carrier for the pigment is evaporated off and the pigment is allowed to seep into the wax layer 11 and be absorbed thereby. Thus, upon cooling, the wax on the transfer medium again solidifies over the pigment layer 12 which is held just below the wax surface. Thus the pigment layer is insulated against contact during handling in that it is overcoated by the solidified wax. Likewise it is insulated against contact with the foundation sheet in that it has not penetrated completely through the wax layer to the foundation sheet as shown by FIG. 1 of the drawing.

Upon the application of pressure against the back of the transfer medium as by a pen, pencil, type bar or sty-

## 2

lus, an image transfers to a copy sheet 20 and is smudge-proof in that it has no pigment at its surface, the surface of the image being the portion of the transfer layer which was adjacent the foundation on the transfer sheet. The surface of the image is thus of clear wax and the pigment layer 12 is held beneath this surface, as shown by FIG. 2 of the drawing. The use of temperatures in the range of 150°—250° F. is necessary to insure that the wax softens or melts to just the right degree to allow the pigment to be absorbed and covered thereby. The duration of the heating depends upon the melting point of the wax layer employed and the temperatures used, but in general, heating continues for only that period of time required for the sheet to pass the heating element at the normal speed of a coating machine.

In another form of the invention, a non-volatile plasticizing agent is added to the pigment dispersion. After application of the pigment dispersion to the wax layer and heating to fusion, the plasticizing agent causes the pigment to wet down and blend or commingle at the interface with the wax layer. Sheets and ribbons prepared in this manner have increased properties of dry rub and the transferred images have increased resistance to smudging. Plasticizing agents comprising oils such as vegetable oils; polyalkylene glycols such as water-insoluble polybutylene glycol; and esters such as butyl stearate and tricresyl phosphate provided excellent results.

In still another form of the present invention, a bonding agent is added to the pigment dispersion with or without the plasticizing agent and it aids in the formation of a better dispersion, mixed for instance in a Waring Blender. The dispersion is coated on the wax layer and heated or fused in the described manner. This heating brings about commingling at the interface thereby providing a relatively hard surface having the pigment well sealed, both by the bonding agent and by the wax underlayer. Apparently the underlayer admixes with the bonding agent so that an exceptionally clean sheet results. As the bonding agent, any material may be used which is at least partially miscible with the wax layer of the foundation. Resinous materials such as ethyl cellulose, methyl cellulose and hydroxyethyl cellulose may be used. Also, any frangible wax, such as those employed in the wax layer of the foundation, as well as spermaceti or cetyl alcohol, may be used successfully. It is preferred that the bonding agent be not only miscible with the wax underlayer but also at least partly soluble in the vehicle for the pigment, such as alcohol, water, petroleum naphtha or ethyl acetate, for instance. In this respect, ethyl cellulose is preferred as the bonding agent with ethanol as the solvent. It should be noted that when a water-soluble binder is used with water as the solvent, conventional wetting agents such as Aerosol AY should be added.

In still a further embodiment of the present invention, the wax layer on the foundation sheet may be pigmented in the conventional manner prior to its application to the paper. It has been found for instance that if the wax layer is pigmented with a blue or other light colored pigment such as titanium dioxide or other white pigment, and then fusion coated with a black or other dark colored pigment, the transfer medium has an appearance much lighter than if the blue or white and black were mixed as one, but the image transferred under pressure has a color darker than would have been expected from the light appearance of the transfer sheet. This appears to be due to a blending or coalescing of the pigments under pressure. Quite unexpectedly, in the case where white pigment is employed in the wax layer, it has been found that the formed transfer sheet is capable of duplicating on black or white copy sheets. When duplicating for instance onto a white copy sheet the formed im-

age appears black, apparently due to a blending of the white pigment of the image with the white background. When duplicating with the same transfer sheet onto a black copy sheet, the formed image appears white, apparently due to a blending of the black pigment of the image with the black background. This feature is quite important, for instance, in the preparation of debit-credit sheets wherein either the debit or credit column is given a black background. Thus, while using only a single transfer sheet, the credit items appear on the receipt or copy sheet in black while the balance or debit items appear in white, or vice versa. Likewise it has been found that titanium dioxide or other white pigment may be incorporated in the wax layer on the foundation sheet and magnetic iron oxide or other magnetic pigment may be applied by the fusion method. Upon transference, the white pigment covers the magnetic iron oxide so that the image itself is hidden or appears quite light but remains magnetically sensible in very way.

The following examples are set forth by way of illustration and should not be considered as limitative.

#### Example I

This example shows the basic step of applying an unmodified pigment dispersion to a wax coated sheet. The steps are as follows.

(1) Ordinary kraft paper is coated with a conventional thickness of a layer of a wax composition having the following recipe:

|                            | Percent |
|----------------------------|---------|
| Carnauba wax               | 30.0    |
| Raw montan wax             | 1.5     |
| Beeswax                    | 2.6     |
| Lanolin                    | 3.0     |
| Mineral oil                | 15.0    |
| Indopol H-300              | 2.4     |
| Lecithin                   | 0.5     |
| Clay                       | 35.0    |
| Pigment (titanium dioxide) | 10.0    |

(2) This wax coated paper is then coated on its wax surface with a pigment dispersion such as graphite dispersed in alcohol. The amount of graphite used depends upon the tone-strength desired in the transfer sheet and adjustments are well within the purview of one skilled in the art.

(3) Some of the product of step 2 is then heated to a temperature of 100° F. to drive off the alcohol solvent. Upon cooling, this transfer sheet is useless in that the graphite merely lies on the wax surface and rubs off when the sheet is handled.

(4) The remainder of the product of step 2 is now steam heated to a temperature of 212°-230° F. for a short period of time to allow the wax to fuse and absorb the graphite. Heating is stopped and the sheet allowed to cool. The transfer sheet is clean to the touch and yields smudge-proof images under pressure.

#### Example II

This example illustrates the use of a binder-containing pigment dispersion, a plastic foundation material and magnetic pigment.

(1) A thin sheet of polyethylene terephthalate (Mylar) film having a thickness of 0.5 mil is overcoated with a layer of pressure-transferable wax of the following formulation:

|                | Percent |
|----------------|---------|
| Carnauba wax   | 54.5    |
| Raw montan wax | 2.8     |
| Beeswax        | 4.7     |
| Lanolin        | 5.6     |
| Mineral oil    | 27.5    |
| Lecithin       | 0.9     |
| Indopol H-300  | 4.0     |

(2) The wax coated Mylar is then coated with a pigment dispersion of magnetic iron oxide and alcohol con-

taining ethyl cellulose binder in about the following proportions:

|                     | Percent |
|---------------------|---------|
| Magnetic iron oxide | 39.3    |
| Alcohol (ethanol)   | 58.7    |
| Ethyl cellulose     | 2.0     |

(3) The product of step 2 above is steam heated to a temperature of 220°-230° F. for a few minutes to allow the wax to melt and absorb the wetted pigment.

10 After cooling, the transfer sheet has excellent qualities of cleanliness and the formed image is smudge-free and completely sensible to magnetic sensing means.

#### Example III

15 This example shows the use of a binder in the pigment dispersion of Formulation 1 and a plasticizer in the pigment dispersion of Formulation 2 as defined below.

20 (1) Conventional kraft paper is coated with wax as in step 1 of Example I.

(2) The wax coated paper of step 1 above is then separated into two portions. These portions are then individually coated on their wax surfaces with a thin coating of a dispersed composition of the following respective formulations.

|                   | Percent |
|-------------------|---------|
| Formulation 1:    |         |
| Carbon black      | 1       |
| Alcohol (ethanol) | 98      |
| Ethyl cellulose   | 1       |

|                                                        | Percent |
|--------------------------------------------------------|---------|
| Formulation 2:                                         |         |
| Graphite or carbon black                               | 1       |
| Alcohol (ethanol)                                      | 90      |
| Dow Polyol B-500 (water-insoluble polybutylene glycol) | 9       |

(3) The individual sheets each coated with these different pigment dispersions are then heated to a temperature between 220°-230° F. for a short period of time to allow the wax layer on the foundation sheet to melt and absorb the binder-containing pigment dispersion. Upon cooling, these transfer sheets are completely clean to the touch, light in appearance and upon transfer the formed image is dark colored and smudge-free.

45 The materials and proportions set forth in these examples are merely illustrative and variations may be made according to the knowledge of the art. For instance, any of the conventional waxes of the animal, vegetable, mineral or synthetic variety may be substituted for those of the examples and the proportions may be varied according to hardness or tackiness desired in the final product.

55 As the pigment dispersion, it has been found convenient to use commercially available dispersions of carbon black or graphite in water-insoluble polyalkylene glycols such as DAG-197 which is a 10% dispersion of graphite in water-insoluble polybutylene glycol manufactured by the Acheson Colloids Company. Likewise a 20% dispersion of graphite in isopropanol, available from Acheson Colloids Company under the name DAG-154, may be used. 60 Alternatively the pigment dispersion may be compounded by mixing the desired pigment in the desired amount with Dow Polyol B-500 which is a water-insoluble polyalkylene glycol.

65 Also, in place of the pigments named, hectograph dyes such as crystal violet or planographic pigments such as nigrosine black and Bismarck brown may be employed.

Variations and modifications may be made within the scope of the claims and portions of the improvements may be used without others.

70 I claim:

1. The method of preparing transfer sheets which are clean to the touch which comprises the steps of coating a foundation sheet with a layer of pressure-transferable wax, applying to the wax surface a dispersion of a pigment, a non-volatile plasticizing agent for said wax and a

volatile carrier, heating to a temperature sufficiently high to cause the wax to soften, allow the pigment to be absorbed thereby and evaporate the volatile carrier, and then cooling to form the transfer sheet in which the pigment is held just below the wax surface and is overcoated by the cooled, solidified wax.

2. The method of claim 1 in which the layer of pressure-transferable wax, prior to application of the pigment dispersion, contains a pigment different from that of said pigment dispersion.

3. The method of claim 1 in which the pigment comprises magnetic pigment.

4. The method of claim 1 in which the plasticizing agent comprises a water-insoluble polyalkylene glycol.

5. The method of claim 1 in which the temperature of heating ranges from 150° F. to 250° F.

6. The method of preparing transfer sheets which are clean to the touch which comprises the steps of coating a foundation sheet with a layer of pressure-transferable wax, applying to the wax surface a dispersion of a pigment, a volatile carrier and a binding agent which is soluble in said carrier, heating to a temperature sufficiently high to soften the wax layer, allow the pigment to be absorbed thereby and evaporate the volatile carrier, and then cooling to form the transfer sheet in which the pigment is held just below the wax surface and is over-

15

20

25

coated by the cooled, solidified wax and said binding agent.

7. The method of claim 6 in which a non-volatile plasticizing agent is present in the pigment dispersion.

8. The method of claim 6 in which the binding agent comprises ethyl cellulose.

9. The method of claim 6 in which the pigment comprises magnetic pigment.

10. The method of claim 6 in which the foundation sheet is a plastic film.

11. The method of claim 6 in which the temperature of heating ranges from 150° F. to 250° F.

References Cited in the file of this patent

UNITED STATES PATENTS

|           |               |               |
|-----------|---------------|---------------|
| 1,189,939 | Goldsmith     | July 4, 1916  |
| 1,864,097 | Sherman       | June 21, 1932 |
| 1,925,235 | Dixon         | Sept. 5, 1933 |
| 2,063,226 | Braunstein    | Dec. 8, 1936  |
| 2,744,031 | Mumma         | May 1, 1956   |
| 2,912,344 | Newman et al. | Nov. 10, 1959 |

FOREIGN PATENTS

|         |               |               |
|---------|---------------|---------------|
| 393,904 | Great Britain | June 15, 1933 |
|---------|---------------|---------------|